

Aug. 20, 1968

A. J. J. HENDRICKX  
LIGHT SENSITIVE DIAZOTYPE MATERIAL AND  
DIAZONIUM COMPOUNDS THEREFOR

3,397,985

Filed Dec. 31, 1964

2 Sheets-Sheet 1

FIG. 1.



FIG. 2.



FIG. 3.



FIG. 4.



FIG. 5.



FIG. 6.



FIG. 7.



INVENTOR

ANDREAS J. J. HENDRICKX

BY

*Albert C. Johnston*

ATTORNEY

Aug. 20, 1968

A. J. J. HENDRICKX

3,397,985

LIGHT SENSITIVE DIAZOTYPE MATERIAL AND  
DIAZONIUM COMPOUNDS THEREFOR

Filed Dec. 31, 1964

2 Sheets-Sheet 2

FIG. 8.



FIG. 9.



INVENTOR

ANDREAS J. J. HENDRICKX

BY

*Albert C. Johnston*

ATTORNEY

**1**

3,397,985

**LIGHT SENSITIVE DIAZOTYPE MATERIAL AND DIAZONIUM COMPOUNDS THEREFOR**

Andreas Joseph Johannes Hendrickx, Venlo, Netherlands, assignor to Van der Grinten N.V., Northern Limburg, Netherlands

Filed Dec. 31, 1964, Ser. No. 422,693

Claims priority, application Netherlands, June 1, 1964, 6406149

9 Claims. (Cl. 96—91)

**ABSTRACT OF THE DISCLOSURE**

Diazotype materials yielding high-contrast azo-dyestuff images on more brightly bleached-out (whiter) backgrounds and having high coupling activity, good light-sensitivity and improved keeping qualities are obtained by providing in the light-sensitive layer a new benzene diazonium salt having a pyrrolidin(2)yl group ortho to the diazonium group, an acylamino or a thio group para thereto, and an ether group para to the pyrrolidin(2)yl group.

The invention relates to diazotype material containing a benzene diazonium salt of a new type and more particularly to one-component diazotype material which is very suitable for development according to the so-called thin layer method with weakly acid buffered developing liquids commonly used in the one-component diazotype process.

In this specification reference is made to the structural chemical formula of compounds. These formulae are set out in the accompanying drawings and the references herein are to the figures of these drawings.

Diazotype materials can be distinguished into: one-component diazotype materials, which are developed with the aid of a liquid containing an azo-coupling component; two-component diazotype materials, which are developed with the aid of gaseous alkali (ammonia); heat-developable diazotype materials; planographic printing plates sensitized with diazo compounds.

One-component diazotype material is usually developed by spreading (after imagewise exposure) a thin layer (4–12 g./m.<sup>2</sup>) of an aqueous developing liquid on the sensitized surface (and also on the non-sensitized surface, if desired).

The developing liquids commonly used in the one-component diazotype process are usually distinguished into alkaline liquids having a pH above 7 and buffered weakly acid liquids the pH of which is between 5.5 and 7. Because of their high keeping quality the weakly acid developers are to be preferred to the alkaline developers. In fact, in diazotype developers phloroglucinol, which in alkaline medium is readily oxidized by the oxygen from the air, is practically always used as azo-coupling component. Developers, both alkaline and buffered weakly acid developers, which contain phloroglucinol as azo-coupling component, often in combination with a quantity of resorcinol, are used on a large scale in practice.

In diazotype materials which can be developed with a weakly acid buffered developer, various diazo compounds derived from hydroquinone dialkyl and diaralkyl ethers and having high coupling activity are employed. Groups of such diazo compounds are: those with the general

5

10

15

20

25

30

35

40

45

50

55

60

**2**

formula according to FIGURE 1, in which X is an anion, R<sub>1</sub> and R<sub>2</sub> are alkyl or aralkyl groups, R<sub>3</sub> stands for a substituted or a non-substituted alkyl, aralkyl, aryl, alkoxy, aralkoxy, aryloxy, a substituted amidocarbonyl or a substituted amido radical, and R<sub>4</sub> for a hydrogen atom or an alkyl group or is an alkyl or acyl group which forms a heterocyclic ring with N—CO—R<sub>3</sub>. (See: British patent specifications Nos. 347,430, 615,774, 539,031, 510,874, 449,341, 520,304, 620,038, 538,869 and 643,309); those with the general formula according to FIGURE 2, in which R<sub>4</sub> stands for a hydrogen atom, an alkyl, aralkyl, or aryl group (see: U.S. patent specification No. 2,665,985); those with the general formula according to FIGURE 3, in which R<sub>5</sub> stands for a substituted or a non-substituted alkyl, aralkyl, or aryl group (see: Fiat Final Report 813, pages 137 and 138, Dutch patent specification No. 51,536, British patent specification No. 759,045 and German patent specification No. 896,591); and those with the general formula according to FIGURE 4, in which R<sub>6</sub> stands for hydrogen, an acetylamino group, a light alkyl or alkoxy group (see: British patent specification No. 471,614).

The diazo compounds according to the formulae of FIGURES 1–4 upon exposure yield a somewhat stained photo-decomposition product, so that copies made on a diazotype material sensitized with such a compound show a stained background. When the support of the diazotype material is white paper, the background of the copies instead of being bright white, shows a somewhat dingy stain; when the support is transparent, the copies—even if the azo-dyestuff image has high absorption for ultra-violet radiation—are not very suitable as intermediate originals for making further copies on diazotype material, because the presence of the stained photo-decomposition product in the image-free portions of the intermediate original decreases its transparency to the ultra-violet copying radiation, and thus necessitates a longer exposure time when further copies are to be made.

Dutch patent application No. 288,469, not previously published, describes diazotype material which contains a diazo compound of the general formula according to FIGURE 5, in which X is an anion, R<sub>1</sub> stands for an alkyl, branched alkyl, cycloalkyl, or aralkyl group, CO—R<sub>2</sub> for an acyl radical, R<sub>3</sub> for a substituent from the group formed by acylamido, alkylsulfonamido, aralkylsulfonamido, arylsulfonamido, and triazinyl radicals, and R<sub>4</sub> for an alkyl, branched alkyl, cycloalkyl, aralkyl, or aryl radical.

Dutch patent application No. 295,561, not previously published, described diazotype material which contains a diazo compound of the general formula according to FIGURE 6, in which X is an anion, R<sub>1</sub> stands for an alkyl, branched alkyl, cycloalkyl, or aralkyl group, CO—R<sub>2</sub> for an acyl radical, R<sub>3</sub> for a saturated or non-saturated organic radical, including the cyano radical, and R<sub>4</sub> for an alkyl, branched alkyl, cycloalkyl, aralkyl, or aryl radical.

The diazotype materials according to the Dutch patent applications Nos. 288,469 and 295,561 have a higher developing speed than diazotype material which has been sensitized with a similar diazo compound, derived from hydroquinone, according to the formulae of FIGURES 1–4, and they are often more light-sensitive as well, particularly when R<sub>1</sub> is a small alkyl group.

The present invention relates to diazotype material

characterized in that it contains a diazo compound of the general formula according to FIGURE 7, in which X is an anion, R stands for an alkyl (i.e., a non-branched or branched alkyl), alkenyl, cycloalkyl, aralkyl, or aryl group, and Y for a substituent from the group formed by acylamino, etherified mercapto, dihydrotriazinyl, and substituted or non-substituted phenyl groups.

In this connection by acylamino is to be understood that radical



in which R<sub>1</sub> stands for an organic radical and R<sub>2</sub> for a hydrogen atom, an alkyl or aralkyl group, or for an alkyl or acyl radical which forms a heterocyclic ring with N-CO-R<sub>1</sub>.

As compared with diazotype material which has been sensitized with a similar diazo compound derived from hydroquinone, the diazotype material according to the invention shows higher light-sensitivity, while moreover it bleaches out brighter.

As compared with the comparable diazotype materials described in the Dutch patent application Nos. 288,469 and 295,561, the diazotype material according to the invention is a little more light-sensitive and as a rule has better keeping quality. Besides, it bleaches out brighter.

The fact that the diazotype material according to the invention bleaches out bright is manifest when the material, while being printed, has a high moisture content, for instance because it has been kept in a humid atmosphere for some hours. Thus copies made of diazotype paper according to the invention, which has been left unpacked, e.g., for an hour in an office room having a temperature of 20° C. and a relatively humidity of 75% before the copies were made, show a much whiter background than copies on diazotype materials sensitized with diazo compounds according to the formulae of FIGURES 1-6 and stored under the same conditions.

The diazotype material according to the invention is preferably one-component diazotype material. Upon development with weakly acid phloroglucinol developers it yields properly developed copies with strong red to very dark-brown azo-dyestuff images. (Of course, one-component diazotype material according to the invention can be developed with weakly alkaline developing liquids; copies also showing strong, somewhat lighter, red to brown azo-dyestuffs are then obtained). The diazotype material according to the invention may also be heat-developable diazotype material.

Whatever may be the composition of the F(nxe)coing

Whatever may be the composition of the material and the method of development, if the azo-dyestuffs formed upon development are sufficiently oleophilic and if the support has the appropriate constitution the copies can be used as a planographic printing form.

Diazo compounds which can be used in the diazotype material according to the invention are:

- 4-diazo-2-methoxy-5-pyrrolidone(2)yl(1)-N-acetyl-aniline  
 4-diazo-2-ethoxy-5-pyrrolidone(2)yl(1)-N-ethoxy-carbonylaniline  
 4-diazo-2-benzyloxy-5-pyrrolidone(2)yl(1)-N-butyryl-aniline  
 4-diazo-2-(4'-chlorobenzyl)oxy-5-pyrrolidone(2)yl(1)-N-acetyl-aniline  
 4-diazo-2-methoxy-5-pyrrolidone(2)yl(1)-N-chloro-acetyl-aniline  
 4-diazo-2-(2'-ethylbutyl)oxy-5-pyrrolidone(2)yl(1)-N-phenacetyl-aniline
- 4
- 4-diazo-2-methoxy-5-pyrrolidone(2)yl(1)-N-benzyloylaniline  
 5-methoxy-2,4-di-pyrrolidone(2)yl(1)-diazobenzene  
 4-diazo-2-methoxy-5-pyrrolidone(2)yl(1)-N-methyl-  
 5 N-benzyloylaniline  
 4-diazo-2-ethoxy-5-pyrrolidone(2)yl(1)-N-benzyloylaniline  
 4-diazo-2-n-propoxy-5-pyrrolidone(2)yl(1)-N-benzyloylaniline  
 10 4-diazo-2-n-butoxy-5-pyrrolidone(2)yl(1)-N-benzyloylaniline  
 4-diazo-2-isocamylloxy-5-pyrrolidone(2)yl(1)-N-benzyloylaniline  
 4-diazo-2-(2'-hydroxyethyl)oxy-5-pyrrolidone(2)yl(1)-N-benzyloylaniline  
 15 4-diazo-2-ethoxyethoxy-5-pyrrolidone(2)yl(1)-N-benzyloylaniline  
 4-diazo-2-(2'-diethylaminoethoxy-5-pyrrolidone(2)yl(1)-N-benzyloylaniline  
 20 4-diazo-2-(4'-chlorophenyl)oxy-5-pyrrolidone(2)yl(1)-N-benzyloylaniline  
 4-diazo-2-allyloxy-5-pyrrolidone(2)yl(1)-N-benzyloylaniline  
 4-diazo-2-cyclopentenoxy-pyrrolidone(2)yl(1)-N-benzyloylaniline bis-N,N'-4'-diazo-2'-methoxy-5'-  
 25 pyrrolidone(2)yl(1)-phenyl)urea  
 1-(4'-diazo-2'-methoxy-5'-pyrrolidone(2)yl(1)-phenyl)-4[2]-amino-2-[4]-imino-6-methyl-  
 1H,2H[1H,4H]1,3,5-triazine  
 30 4-diazo-2-methoxy-5-pyrrolidone(2)yl(1)-phenylthiomethyl ether  
 4-diazo-2-ethoxy-5-pyrrolidone(2)yl(1)-phenylthiomethyl ether  
 4-diazo-2-n-propoxy-5-pyrrolidone(2)yl(1)-  
 35 phenylthiomethyl ether  
 4-diazo-2-n-butoxy-5-pyrrolidone(2)yl(1)-phenylthiomethyl ether  
 4-diazo-2-methoxy-5-pyrrolidone(2)yl(1)-phenylthioethyl ether  
 40 4-diazo-2-ethoxy-5-pyrrolidone(2)yl(1)-phenylthioethyl ether  
 4-diazo-2-n-propoxy-5-pyrrolidone(2)yl(1)-phenylthioethyl ether  
 4-diazo-2-allyloxy-5-pyrrolidone(2)yl(1)-phenylthioethyl ether  
 45 4-diazo-2-n-butoxy-5-pyrrolidone(2)yl(1)-phenylthioethyl ether  
 4-diazo-2-(4'-chlorophenyl)oxy-5-pyrrolidone(2)yl(1)-phenylthioethyl ether  
 50 4-diazo-2-cyclopentenoxy-5-pyrrolidone(2)yl(1)-phenylthioethyl ether  
 4-diazo-2-methoxy-5-pyrrolidone(2)yl(1)-phenylthiobutyl ether  
 4-diazo-2-(2'-ethylbutyl)oxy-5-pyrrolidone(2)yl(1)-phenylthiocarboxymethyl ether  
 55 4-diazo-2-benzyloxy-5-pyrrolidone(2)yl(1)-phenylthiobenzyl ether  
 ethanedithiol-(1,2)-bis(4'-diazo-2'-methoxy-5'-  
 pyrrolidone(2)yl(1)-phenyl) ether  
 60 4-diazo-2-methoxy-5-pyrrolidone(2)yl(1)-phenylthio-p-tolyl ether  
 4-diazo-2-ethoxy-5-pyrrolidone(2)yl(1)-phenylthio-p-tolyl ether  
 4-diazo-2-n-propoxy-5-pyrrolidone(2)yl(1)-phenylthio-  
 65 p-tolyl ether  
 4-diazo-2-n-butoxy-5-pyrrolidone(2)yl(1)-phenylthio-p-tolyl ether  
 4-diazo-2-(4'-chlorophenyl)oxy-5-pyrrolidone(2)yl(1)-phenylthio-p-tolyl ether  
 70 4-diazo-2-methoxy-5-pyrrolidone(2)yl(1)-diphenyl  
 4-diazo-2-ethoxy-5-pyrrolidone(2)yl(1)-diphenyl  
 4-diazo-2-n-propoxy-5-pyrrolidone(2)yl(1)-  
 diphenyl  
 4-diazo-2-n-butoxy-5-pyrrolidone(2)yl(1)-  
 diphenyl

- 4-diazo-2-cyclopentoxy-5-pyrrolidon(2)yl(1)-  
diphenyl  
4-diazo-2,4'-dimethoxy-5-pyrrolidon(2)yl(1)-  
diphenyl  
4-diazo-2-n-butoxy-4'-methoxy-5-pyrrolidon(2)yl(1)-  
diphenyl.

The diazo compounds are used as diazonium salts, for instance as chlorides or sulfates, or as diazonium metal double salts, such as the zinc chloride double salt, the manganese chloride double salt, and the stannic chloride double salt, or as borofluorides. They can be applied separately, mixed together, or in admixture with diazo compounds of other types. It is obvious that, when mixtures are used, the effect of the new diazo compounds will be smaller according as a larger quantity of the other compound(s) is used.

Although the diazo compounds according to the invention have high coupling activity and good light-sensitivity, moreover bleach out while forming practically colourless photo-decomposition products, and yield high-contrast azo-dyestuffs with the conventional azo-coupling components, such as phloroglucinol and resorcinol, nevertheless there are differences in qualities and accessibility between the various diazo compounds.

Because of their ready accessibility, their comparatively very high coupling activity, and their relatively high stability, the diazo compounds having a benzoylamino or an etherified mercapto group in para-position relative to the diazo group are preferred. Diazotype materials which have good keeping quality, develop very rapidly, and are reasonably inexpensive can be prepared with these diazo compounds.

Very useful compounds are, for instance, those of the general formula according to FIGURE 8 in which  $R_1$  represents a non-branched alkyl group having up to 5 carbon atoms and X represents an anion.

Particularly valuable diazo compounds are those with an alkyl, aralkyl, or arylthio group in para-position and more especially those of the general formula according to FIGURE 9, in which  $R_1$  represents a non-branched alkyl group having up to 5 carbon atoms,  $R_2$  represents a non-branched alkyl group having up to 4 carbon atoms or a substituted or non-substituted benzyl or phenyl group, and X represents an anion.

Diazotype material sensitized therewith has higher light-sensitivity than diazotype material according to the invention containing a diazo compound with another substituent in para-position.

In the diazotype material according to the invention, the support to be used may be paper, printing-plate paper, tracing paper, transparentized paper, linen, tracing linen, synthetic paper, film material, such as films of cellulose acetate and polyester, metal, e.g. planographic printing plates of aluminium.

Furthermore the diazotype material according to the invention may contain the additions commonly used in the diazotype process, e.g. acids, such as citric acid, tartaric acid, and boric acid; stabilizers, such as benzene and naphthalene sulfonic acids and their water-soluble salts, e.g. sodium naphthalene 1,3,6-trisulfonate; metal salts, such as zinc chloride, magnesium chloride, nickel sulfate, and alum; surface-improving substances, such as finely divided silica (colloidal or non-colloidal), aluminium oxide, barium sulfate, rice starch, etc.; binders, such as gelatin, gum arabic, cellulose ethers, starch derivatives, polyvinyl alcohol; dispersions of synthetic resins, such as dispersions of polyvinyl acetate in aqueous media containing cationic, non-ionic or anionic dispersing agents.

The phloroglucinol developers which are used in the one-component diazotype process often vary as to their composition and acidity. Below three weakly acid phloroglucinol developers employed in practice are described. These developers will be used for development in the following examples.

Developer A is a solution of:

|    |                                                                                                                                    |    |     |
|----|------------------------------------------------------------------------------------------------------------------------------------|----|-----|
| 5  | Phloroglucinol                                                                                                                     | g  | 4   |
|    | Acetoacetanilide                                                                                                                   | g  | 0.1 |
| 10 | 2-ethyl-1-hexanol sulfate Tergitol 08 (from Union Carbide & Carbon Corp., New York 17, U.S.A.; Tergitol is a registered trademark) | ml | 3   |
|    | Beet sugar                                                                                                                         | g  | 15  |
|    | Benzoic acid                                                                                                                       | g  | 2.5 |
| 15 | Sodium benzoate                                                                                                                    | g  | 14  |
|    | Sodium formate                                                                                                                     | g  | 135 |

in 1000 ml. of water.

The pH of this liquid is approximately 5.8.

Developer B is a solution of:

|    |                                                                                                                                      |    |     |
|----|--------------------------------------------------------------------------------------------------------------------------------------|----|-----|
| 20 | Phloroglucinol                                                                                                                       | G. | 6.5 |
|    | Resorcinol                                                                                                                           |    | 4   |
| 25 | Thiourea                                                                                                                             |    | 10  |
|    | Sodium butylnaphthalene sulfonate Sorbit P (from Geigy Chem. Corp. Ardsley, N.Y., U.S.A.; the word Sorbit is a registered trademark) |    | 2   |
|    | Sodium formate                                                                                                                       |    | 14  |
|    | Sodium benzoate                                                                                                                      |    | 22  |
| 30 | Trisodium citrate (2 aq.)                                                                                                            |    | 49  |
|    | Citric acid                                                                                                                          |    | 1.2 |

in 1000 ml. of water.

The pH of this liquid is 6.5.

Developer C is a solution of:

|    |                                       |    |    |
|----|---------------------------------------|----|----|
| 35 | Phloroglucinol                        | g  | 5  |
|    | Resorcinol                            | g  | 1  |
|    | Dipotassium phosphate                 | g  | 3  |
|    | Tergitol 08                           | ml | 3  |
|    | Maleic anhydride                      | g  | 52 |
|    | Potassium hydroxide solution (13.5 N) | ml | 75 |

40 in 1000 ml. of water.

The pH of this liquid is 6.9.

In addition to phloroglucinol (and in addition to, or instead of, resorcinol), the weakly acid buffered developers may also contain other azo-coupling components having high coupling activity, e.g. 2,3 - dihydroxynaphthalene, and acetoacetanilide.

The following examples will serve to illustrate the invention:

#### Example I

50 Three sensitizing liquids are prepared:

(A) A liquid containing:

|    |                                                                                                        |      |
|----|--------------------------------------------------------------------------------------------------------|------|
| 55 | 4-benzoylamino - 2 - pyrrolidon(2)yl(1)-5-methoxybenzene diazonium chloride, zinc chloride double salt | 16.6 |
|    | Tartaric acid                                                                                          | 5    |
|    | Saponin                                                                                                | 3    |

60 in 1000 ml. of water.

(B) A similar liquid to that mentioned under (A), but containing, instead of the 4-benzoylamino-2-pyrrolidon(2)yl(1)-5-methoxybenzene diazonium salt, and equimolar quantity of 4-benzoylamino-2-N-methyl-N-acetyl-amino-5-methoxybenzene diazonium chloride, zinc chloride double salt.

(C) A similar liquid to that mentioned under (A), but containing, instead of the said diazonium salt, an equimolar quantity of 4-benzoylamino-2,5-dimethoxybenzene diazonium chloride, zinc chloride double salt.

With each of these liquids a sheet of white base paper of weight 80 g./m.<sup>2</sup> and suitable for the diazotype process is sensitized. After sensitization the three sheets are dried. Each sheet contains approximately 0.40 millimol of diazo compound per m.<sup>2</sup>. A strip of each sheet is imagewise ex-

posed underneath a transparent ink drawing for the time required to bleach out, on the strip of sheet (A), all the diazo compound underneath the image-free portions of the original. After this, the strips are developed with developer (A).

Strip (A) shows a violet-brown image on a bright white background. Strip (B) shows a dark brown image on a somewhat foggy background, and strip (C) shows a black image on a heavy violet-grey background.

A second strip of the sheets (A), (B) and (C), screened from the light, is kept for an hour in a room having a relative humidity of 75% and a temperature of approximately 20° C. The strips are then fed, together with a transparent ink drawing, through a continuously operating exposure apparatus for the diazotype process comprising an exposure cylinder of glass which has a surface temperature of approximately 60° C. and in which a high-pressure mercury vapour lamp is mounted, with such a speed that, on strip (C), all the diazo compound underneath the image-free portions of the drawing has bleached out.

The strips are then developed with developer (A). It is clearly visible that the "white" background of the strips (B) and (C) is less white than that of strip (A).

The 2-pyrrolidon(2)yl(1) diazo compound used in the example was prepared as follows: p-aminophenol was brought into reaction with  $\gamma$ -butyrolactone. Thus 4-pyrrolidon(2)yl(1)phenol was formed, which product was nitrated and then methylated with dimethyl sulfate. The nitro group was reduced to an amino group and the amino group was benzoylated. The 4-pyrrolidon(2)yl(1)-2-benzoylaminooanisole was nitrated to 4-pyrrolidon(2)yl(1)-2-benzoylaminoo-5-nitroanisole, which melts at 223-225° C. Upon reduction, 4-benzoylaminoo-2-pyrrolidon(2)yl(1)-5-methoxyaniline was formed, which product was diazotized. The diazo compound was obtained in the form of the chlorozincate.

## EXAMPLE II

White base paper of weight 80 g./m.<sup>2</sup> and suitable for the diazotype process is sensitized with a liquid containing:

| G.                                                                                                 |    |
|----------------------------------------------------------------------------------------------------|----|
| 4 - phenyl - 2 - pyrrolidon(2)yl(1)-5-methoxybenzene diazonium chloride, zinc chloride double salt | 15 |
| Tartaric acid                                                                                      | 5  |
| Saponin                                                                                            | 3  |

in 1000 ml. of water and dried.

The diazotype paper thus obtained contains approximately 0.45 millimol of diazo compound per m.<sup>2</sup>. A sheet of the diazotype paper is imagewise exposed underneath a transparent ink drawing until all the diazo compound underneath the image-free portions of the drawing has bleached out, and is then developed with developer (A).

The copy shows a red image on a bright white background.

When the above-mentioned sensitizing liquid contains, instead of the said diazo compound, an equimolar quantity of the diazo compound 4-phenyl-2,5-dimethoxybenzene diazonium chloride, zinc chloride double salt, the diazotype paper thus obtained is considerably less light-sensitive, and gives copies with a black azo-dye-stuff image on a background having a somewhat dingy stain.

The diazo compound used in the example was prepared as follows: 2-hydroxybiphenyl was methylated and then nitrated. The nitro group of the 2-methoxy-5-nitrobiphenyl was reduced and the amino group thus obtained was brought into reaction with  $\gamma$ -butyrolactone. The 2-phenyl-4-pyrrolidon(2)yl(1)anisole thus prepared was nitrated to 4 - phenyl-2-pyrrolidon(2)yl(1)-5-methoxynitrobenzene, which melts at 123° C. From this nitro compound the diazo compound was prepared by reduction and diazotization; it was obtained in the form of the chlorozincate.

## Example III

Three sensitizing liquids are prepared:  
(A) A liquid containing:

|   |                                                                                                                     |    |
|---|---------------------------------------------------------------------------------------------------------------------|----|
| 5 | 4 - (4' - methylphenylthio)-2-pyrrolidon(2)-yl(1)-5-G. methoxybenzene diazonium chloride, zinc chloride double salt | 16 |
|   | Tartaric acid                                                                                                       | 5  |
|   | Saponin                                                                                                             | 3  |

in 1000 ml. of water.

(B) A similar liquid to that mentioned under (A), but containing, instead of the said diazo compound, an equimolar quantity of 4-(4'-methylphenylthio)-2-N-methyl-N-ethoxycarbonylaminoo-5-methoxybenzene diazonium chloride, zinc chloride double salt.

(C) A similar liquid to that mentioned under (A), but containing, instead of the said diazo compound, an equimolar quantity of 4-(4'-methylphenylthio)-2,5-dimethoxybenzene diazonium chloride, zinc chloride double salt.

With each of these liquids a sheet of white base paper of weight 80 g./m.<sup>2</sup> and suitable for the diazotype process is sensitized. After sensitization the three sheets are dried. Each sheet contains approximately 0.37 millimol of diazo compound per m.<sup>2</sup>.

With each sheet is imagewise exposed underneath a transparent ink drawing for the time required to bleach out on the strip of sheet (A), all the diazo compound underneath the image-free portions of the original. After this, the strips are developed with developer (B).

Strip (A) shows a brown image on a bright white background. Strip (B) shows a dark brown image on a somewhat foggy light brown background. Strip (C) shows a green-black image on a heavily foggy grey background.

A second strip of the sheets (A), (B), and (C), screened from the light, is stored for an hour in a room with a relative humidity of 75% and a temperature of approximately 20° C. The strips are then fed, together with a transparent ink drawing, through a continuously operating exposure apparatus for the diazotype process with an exposure cylinder of glass which has a surface temperature of approximately 60° C. and in which a high-pressure mercury vapour lamp is mounted, with such a speed that on strip (C) all the diazo compound underneath the image-free portions of the drawing has bleached out.

The strips are then developed with developer (B). The "white" background of the strips (B) and (C) is far less white than that of strip (A).

The diazo compound with the 2-pyrrolidon(2)yl(1) group used in the example was prepared as follows: 4-pyrrolidon(2)yl(1) - 2 - nitroanisole was reduced to 5-pyrrolidon(2)yl(1)-2-methoxyaniline. The amino group was replaced according to the Sandmeyer reaction, by a chlorine atom and the product thus formed was nitrated. The chlorine atom was subsequently replaced by a p-tolylthio group with the aid of p-tolylmercaptan. The 4-p-tolylthio - 5-methoxy-2-pyrrolidon(2)yl(1)-nitrobenzene thus obtained melts at 175-176° C. From this nitro compound the diazonium salt was obtained in the usual way.

## Example IV

Paper consisting as to about 50% of synthetic fibres, which has been precoated with an aqueous dispersion of non-colloidal silica and has then been dried, is sensitized with a liquid containing:

| G.                                                                                                                   |    |
|----------------------------------------------------------------------------------------------------------------------|----|
| 4 - phenacylaminoo - 2 - pyrrolidon(2)yl(1)-5-(2'-ethylbut)oxy benzene diazonium chloride, zinc chloride double salt | 22 |
| Tartaric acid                                                                                                        | 5  |
| Saponin                                                                                                              | 3  |

in 1000 ml. of water and dried.

The diazotype paper thus obtained contains approximately 0.37 millimol of diazo compound per m.<sup>2</sup>. The

diazotype paper is imagewise exposed as described in Example II and is then developed with developer (B).

The copy shows a brown image on a non-stained background.

The diazo compound used in the example was prepared as follows: p-aminophenol was brought into reaction with  $\gamma$ -butyrolactone, then nitrated, and alkylated with 2-ethylbutyl bromide to 2-nitro-4-pyrrolidon(2)yl(1)(2'-ethylbut)oxy benzene. The nitro group was reduced to an amino group. The latter was acylated with phenacyl chloride. The product thus obtained was nitrated to 4-phenacylaminio-5-(2'-ethylbut)oxy-2-pyrrolidon(2)yl(1)-nitrobenzene, which melts at 148-151° C. From this nitro compound the diazonium compound was obtained in the usual way.

#### Example V

A celluloseacetate film layer of weight approximately 20 g./m.<sup>2</sup> applied on natural tracing paper of weight about 80 g./m.<sup>2</sup>, is superficially hydrolysed to a depth 20 of about 4 microns and, after removal of the chemicals used for the hydrolysis by washing with water, is sensitized with a solution of

|                                                       | G.  |
|-------------------------------------------------------|-----|
| 4,1'H,2'H[1'H,4'H]-2'[4'] - imino - 4' - [2']-amino-  |     |
| 6' - methyl - 1',1',3',5' - triazinyl-(1')-5-methoxy- |     |
| 2-pyrrolidon(2)yl(1)-benzene diazonium chloride,      |     |
| zinc chlroide double salt -----                       | 120 |
| Tartaric acid -----                                   | 5   |
| Ethanol (96%) -----                                   | 200 |
| Water -----                                           | 800 |

and dried.

The diazotype material thus obtained contains approximately 0.95 millimol of diazo compound per m.<sup>2</sup>. The 35 diazotype material is imagewise exposed as described in Example II and is then developed with developer (B).

The copy shows a dark brown image on a clear background.

The diazo compound used in the example was prepared 40 as follows: 5-pyrrolidon(2)yl(1)-2-methoxyaniline, HCl-salt, was brought into reaction with dicyanodiamide, after which the biguanidino substituent thus introduced was converted with acetic anhydride into a 6-methyl-4,[2]-imino-2,[4]-amino-1H,4H[1H,2H]1,3,5-triazinyl group. The compound thus obtained was nitrated at 4,6'-methyl-4'-[2'] - imino - 2'[4']-amino-1'H,4'H[1'H,2'H]-1',3',5'-triazinyl(1') - 2 - pyrrolidon(2)yl(1)-5-methoxynitrobenzene which melts at 242° C. From this nitro compound the diazonium salt was obtained in the usual way.

#### Example VI

Transparentized paper (grade 506 from Plastic Coating Corporation, Massachusetts, U.S.A.) is sensitized with a liquid containing:

|                                                       |    |
|-------------------------------------------------------|----|
| Bis - N,N'-(4 - diazo - 2 - methoxy - 5 - pyrrolidon- | 37 |
| (2)yl(1)-phenyl)urea, chlorozincate -----             |    |
| Tartaric acid -----                                   | 5  |
| Saponin -----                                         | 3  |

in 1000 ml. of water and dried.

The transparent diazotype paper thus obtained contains approximately 1.18 millimols of diazo compound per m.<sup>2</sup>. A sheet of the diazotype paper is imagewise exposed underneath a typed letter until all the diazo compound underneath the image-free portions of the letter has bleached out, and is then developed with developer (C).

The copy shows a brown azo-dyestuff image on a non-stained background. The azo-dyestuff image has good absorption for ultra-violet radiation, so that the copy is eminently suitable as an intermediate original for making further copies on diazotype material.

The diazo compound used in the example was prepared as follows: 5-pyrrolidon(2)yl(1)-2-methoxyaniline was 75

brought into reaction with phosgene and then nitrated, in consequence of which bis-N,N'-(4-nitro-5-pyrrolidon(2)yl(1)-2-methoxyphenyl)urea was formed, which product melts at 306-307° C. From this bis-nitro compound the bis-diazonium salt was obtained.

#### Example VII

White base paper of weight 80 g./m.<sup>2</sup> and suitable for the diazotype process is sensitized with a liquid containing:

|                                                       |    |
|-------------------------------------------------------|----|
| 4 - diazo - 2 - methoxy - 5 - pyrrolidon(2)yl(1)phen- |    |
| ylthio-n-butyl ether, chlorozincate -----g            | 20 |
| Tartaric acid -----g                                  | 5  |
| Sodium naphthalene 1,3,6-trisulfonate -----g          | 30 |
| Vinnapas H.60 (polyvinyl acetate dispersion from      |    |
| Wacker Chemie G.m.b.H., Munich, Germany; Vin-         |    |
| napas is a registered trademark) -----ml              | 30 |

in 1000 ml. of water and dried.

The diazotype material thus obtained contains approximately 0.45 millimol of diazo compound per m.<sup>2</sup>. A sheet of the diazotype paper is imagewise exposed underneath a typed letter, until all the diazo compound underneath the image-free portions of the letter has bleached out, and is then developed with developer (C).

The copy shows a brown image on a bright white background.

The diazo compound used in the example was prepared as follows: p-nitrophenol was chlorinated to 4-nitro-2-chlorophenol. This product was reduced, brought into reaction with  $\gamma$ -butyrolactone, and then methylated and nitrated. The 2-pyrrolidon(2)yl(1)-5-methoxy-4-chloronitrobenzene thus obtained was converted with butyl-mercaptopan into 4-butylthio-5-methoxy-2-pyrrolidon(2)yl(1)-nitrobenzene, which melts at 99° C. From this nitro compound the diazonium salt was obtained in the usual way.

#### Example VIII

White base paper of weight 80 g./m.<sup>2</sup> and suitable for the diazotype process is sensitized with a solution of

|                                                             |    |
|-------------------------------------------------------------|----|
| Ethane - 1,2 - dithiol - bis -(4' - diazo - 2' - methoxy-   |    |
| 5' - pyrrolidon(2)yl(1) - phenyl)ether, chlorozincate ----- | 25 |
| Tartaric acid -----                                         | 5  |
| Vinnapas H.60 -----                                         | 30 |
| Sodium naphthalene 1,3,6-trisulfonate -----                 | 30 |

in 1000 ml. of water and dried.

The diazotype paper thus obtained contains approximately 0.39 millimol of diazo compound per m.<sup>2</sup>. A sheet of the diazotype paper thus obtained is imagewise exposed and developed as described in Example V.

The copy shows a brown image on a bright white background.

The diazo compound used in the example was prepared as follows: 2-pyrrolidon(2)yl(1)-5-methoxy-4-chloronitrobenzene was brought into reaction with ethane-1,2-dithiol. The ethane-1,2-dithiol-bis-(4'-nitro-2'-methoxy-5'-pyrrolidon(2)yl(1)phenyl) ether thus produced melts at 274-275° C. From this bis-nitro compound the bis-diazonium salt was prepared in the usual way.

#### Example IX

White paper of weight 150 g./m.<sup>2</sup>, coated on one side with a cellulose acetate film layer (approximately 50% by weight of combined acetic acid) of a thickness of approximately 10 microns, which layer has been affixed to the paper by means of an adhesive and has been deacetylated to a depth of about 4 microns to an average acetyl content, calculated as combined acetic acid, of 20% by weight (which corresponds to an average number of acyl groups at the OH-groups of 0.7), is coated on the deacetylated side of the cellulose acetate layer with a liquid containing:

## 11

|                                                                            |     |    |
|----------------------------------------------------------------------------|-----|----|
| Titanium dioxide with a particle size of approximately 0.2 micron          | g.  | 13 |
| Hydroxyethylcellulose Cellosize WP-09 (from Union Carbide Corp. of U.S.A.) | g.  | 27 |
| Glyoxal                                                                    | g.  | 4  |
| Ethanol (96%)                                                              | ml. | 8  |
| Water                                                                      | ml. | 92 |

and dried at 110° C. during 50 seconds.

The layer thus formed is sensitized with a solution of 25 g. of 4-p-tolylthio-5-methoxy-2-pyrrolidon(2)yl(1)-benzene diazonium chloride, zinc chloride double salt in 500 ml. of ethanol (96%) and 500 ml. of water and dried.

The light-sensitive planographic printing plate thus obtained is exposed under a positive original until all the diazo compound underneath the image-free portions of it has bleached out, and the image is subsequently developed by amply wetting the surface of the plate with a liquid which was prepared by dissolving

|                              |     |    |
|------------------------------|-----|----|
| Phloroglucinol               | g.  | 12 |
| Citric acid                  | g.  | 11 |
| Concentrated phosphoric acid | ml. | 87 |

in 950 ml. of water and by bringing the pH of this solution up to 7 with a sodium hydroxide solution.

After development, the plate is washed and mounted in an offset printer, upon which prints can at once be made from the plate.

The background of the plate is bright white and does not absorb fatty printing ink during printing.

## Example X

White baryta-coated paper is sensitized with a solution containing:

|                                                                                                                        |     |     |
|------------------------------------------------------------------------------------------------------------------------|-----|-----|
| 4 - benzylthio - 5 - benzyloxy - 2 - pyrrolidon(2)yl(1)-benzene diazonium chloride, zinc chloride double salt          | g.  | 18  |
| Tartaric acid                                                                                                          | g.  | 5   |
| The aqueous 40% solution of sodium xylene sulfonate Naxonad 4 L (from Nease Chemical Company, Lock Haven, Pa., U.S.A.) | ml. | 5   |
| Ethanol (96%)                                                                                                          | ml. | 500 |
| Water                                                                                                                  | ml. | 500 |

and dried.

The diazotype paper thus obtained contains approximately 0.44 millimol of diazo compound per m.<sup>2</sup>. A sheet of this paper is imagewise exposed as described in Example II and is developed with developer (A).

The copy shows a very dark violet-brown image on a white background.

The diazo compound used in the example was prepared as follows: 4-pyrrolidon(2)yl(1)-2-chlorophenol was benzylated, then nitrated and subsequently brought into reaction with benzylmercaptan. The 4-benzylthio-5-benzyloxy - 2 - pyrrolidon(2)yl(1) - nitrobenzene thus obtained melts at 167° C. From this nitro compound the diazonium salt was obtained in the usual way.

## Example XI

White base paper of weight 80 g./m.<sup>2</sup> and suitable for the diazotype process is coated with a layer by applying approximately 25 g. of a dispersion containing:

|                                                                                                       |     |     |
|-------------------------------------------------------------------------------------------------------|-----|-----|
| Di(octadecylammonium)oxalate                                                                          | G.  | 115 |
| Hydrolysed potato starch, Farinex T.S.D. (from Nationale Zetmeelindustrie N.V., Veendam, Netherlands) | ml. | 35  |
| Gum arabic                                                                                            | g.  | 7.5 |
| Oxalic acid, 2H <sub>2</sub> O                                                                        | g.  | 2.5 |

## 12

in 1000 ml. of water and dried.

A light-sensitive layer is formed on the dried layer by applying a liquid containing:

|                                                                                                            |     |      |
|------------------------------------------------------------------------------------------------------------|-----|------|
| 5 - methylthio - 2 - pyrrolidon(2)yl(1) - 5 - methoxybenzene diazonium chloride, zinc chloride double salt | g.  | 7    |
| 7'-hydroxy-1',2',4,5-naphthimidazole                                                                       | ml. | 20   |
| Tartaric acid                                                                                              | ml. | 22.5 |
| Gum arabic                                                                                                 | g.  | 7.5  |
| Farinex T.S.D.                                                                                             | ml. | 35   |
| Di(octadecylammonium)oxalate                                                                               | ml. | 115  |

in 1000 ml. of water and drying.

The diazotype paper thus obtained contains approximately 0.40 millimol of diazo compound per m.<sup>2</sup>. A sheet of it is exposed underneath a transparent ink drawing until all the diazo compound underneath the image-free portions of the drawing has bleached out. The exposed sheet is developed by bringing it into contact with a surface heated to 150° C.

The copy shows a violet-red image on a bright white background.

The diazo compound used in the example was prepared as follows:

5 - pyrrolidon(2)yl(1)-4-nitro-2-methoxychlorobenzene (see Example III) was brought into reaction with methylmercaptan. The 4-methylthio-5-methoxy-2-pyrrolidon(2)yl(1)-nitrobenzene thus obtained melts at 137-138° C.

From this nitro compound the diazonium salt was obtained in the usual way.

## Example XII

Sized natural tracing paper is sensitized with a solution containing:

|                                                                                                                    |     |     |
|--------------------------------------------------------------------------------------------------------------------|-----|-----|
| 4-N-methyl-N-benzoylamino - 5 - methoxy-2-pyrrolidon(2)yl(1)-benzene diazonium chloride, zinc chloride double salt | g.  | 21  |
| Tartaric acid                                                                                                      | g.  | 5   |
| Ethanol (96%)                                                                                                      | ml. | 100 |
| Water                                                                                                              | ml. | 900 |

and dried.

The transparent diazotype paper thus obtained contains approximately 0.63 millimol of diazo compound per m.<sup>2</sup>. A sheet of this paper is imagewise exposed as described in Example I and is then developed with developer (B).

The copy shows a red image on a clear background.

The diazo compound used in the example was prepared as follows: 2-methylamino-4-nitroanisole was converted with benzoyl chloride into 2-N-methyl-N-benzoylamino-4-nitroanisole. The nitro group of this product was reduced to an amino group, which was brought into reaction with  $\gamma$ -butyrolactone. The 2-N-methyl-N-benzoylamino-4-pyrrolidon(2)yl(1)-anisole thus obtained was nitrated to 4-N-methyl-N-benzoylamino-5-methoxy - 2 - pyrrolidon(2)yl(1)-nitrobenzene, which melts at 137° C. From this nitro compound the diazonium salt was obtained in the usual way.

## Example XIII

White base paper of weight 80 g./m.<sup>2</sup> and suitable for the diazotype process is sensitized with a solution of

|                                                                                                             |     |    |
|-------------------------------------------------------------------------------------------------------------|-----|----|
| 65 4-(4'-methylphenylthio) - 5 - (4'-chlorophenoxy)-2-pyrrolidon(2)yl(1)-benzene diazonium hydrogen sulfate | g.  | 25 |
| Tartaric acid                                                                                               | g.  | 5  |
| Vinnapas H. 60                                                                                              | ml. | 30 |

in 1000 ml. of water and dried.

The diazotype material thus obtained contains approximately 0.40 millimol of diazo compound per m.<sup>2</sup>. A sheet of it is imagewise exposed and developed as described in Example V.

13

The copy shows a dark brown image on a bright white background.

The diazo compound used in the example was prepared as follows: 3,4-dichloronitrobenzene was fused together with p-chlorophenol and potassium hydroxide. As a result 3-chloro-4-p-chlorophenoxynitrobenzene was produced. This product was reduced and then brought into reaction with  $\gamma$ -butyrolactone. The 4-p-chlorophenoxy-3-chloropyrrolidon(2)yl(1)-benzene was nitrated and converted with p-tolylmercaptan into 4-p-tolylthio-5-p-chlorophenoxy-2-pyrrolidon(2)yl(1)-nitrobenzene, which melts at 140-141° C. From this nitro compound the diazonium salt was obtained in the usual way.

What I claim is:

1. Diazotype material comprising a support having thereon a light-sensitive layer containing a benzene diazonium salt of the general formula



in which X represents an anion, R represents an alkyl, alkenyl, cycloalkyl, aralkyl or aryl group, and Y represents an acylamino, etherified mercapto or dihydro-1,3,5-triazinyl group, or a non-substituted or alkyl- or alkoxy-substituted phenyl group.

2. One-component diazotype material according to claim 1, wherein Y is a benzoylamino radical.

3. One-component diazotype material according to claim 1, wherein Y represents an alkyl-thio, aralkyl-thio or aryl-thio group.

4. A diazo compound of the general formula



in which R<sub>1</sub> represents a non-branched alkyl group having up to 5 carbon atoms, and X represents an anion.

14

5. A diazo compound of the general formula



in which R<sub>1</sub> represents a non-branched alkyl group having up to 5 carbon atoms, R<sub>2</sub> represents an alkyl group having up to 4 carbon atoms, a benzyl group or a non-substituted or alkyl- or alkoxy-substituted phenyl group, and X represents an anion.

6. Diazotype material comprising a support having thereon a light-sensitive layer containing a 4-benzoylamino-2-pyrrolidon(2)yl(1)-5-methoxy-benzene diazonium salt.

7. A 4-benzoylamino-2-pyrrolidon(2)yl(1)-5-methoxy-benzene diazonium salt.

8. Diazotype material comprising a support having thereon a light-sensitive layer containing a 4-(4'-methylphenylthio)-2-pyrrolidon(2)yl(1)-5-methoxy-benzene diazonium salt.

9. A 4-(4'-methylphenylthio)-2-pyrrolidon(2)yl(1)-5-methoxy-benzene diazonium salt.

#### References Cited

##### UNITED STATES PATENTS

|           |         |                        |          |
|-----------|---------|------------------------|----------|
| 2,286,701 | 6/1942  | Werner -----           | 96-91    |
| 2,456,514 | 12/1948 | Johnston -----         | 96-91    |
| 2,665,985 | 1/1954  | Sus -----              | 96-91    |
| 3,016,298 | 1/1962  | Sanders et al. -----   | 96-91 XR |
| 3,155,512 | 11/1964 | De Boer -----          | 96-91    |
| 3,338,713 | 8/1967  | Hendrickx et al. ----- | 96-91    |

##### FOREIGN PATENTS

|         |        |                |
|---------|--------|----------------|
| 538,869 | 8/1941 | Great Britain. |
|---------|--------|----------------|

##### OTHER REFERENCES

Brown, D. J.: "Chem. Ind.", 22 (1944), pp. 146-148.

45 NORMAN G. TORCHIN, *Primary Examiner.*

C. L. BOWERS, *Assistant Examiner.*